



US008419870B2

(12) **United States Patent**  
**Coe et al.**

(10) **Patent No.:** **US 8,419,870 B2**  
(45) **Date of Patent:** **Apr. 16, 2013**

(54) **METHOD FOR MAKING STRAIN AGING RESISTANT STEEL**

4,339,284 A 7/1982 Hashimoto et al.  
4,375,376 A 3/1983 Rowden et al.  
4,853,032 A 8/1989 Yalamanchili et al.  
5,342,700 A 8/1994 Arnaud et al.  
5,458,699 A 10/1995 Tsukamoto et al.  
5,556,485 A 9/1996 Taylor et al.  
5,595,617 A 1/1997 Tonteling et al.  
5,656,102 A 8/1997 Taylor et al.  
5,656,103 A 8/1997 Roberts

(75) Inventors: **C. Larry Coe**, Sterling, IL (US); **Alan T. Gorton**, Marietta, GA (US)

(73) Assignee: **L&P Property Management Company**, South Gate, CA (US)

(\*) Notice: Subject to any disclaimer, the term of this patent is extended or adjusted under 35 U.S.C. 154(b) by 28 days.

(21) Appl. No.: **12/761,255**

(22) Filed: **Apr. 15, 2010**

(65) **Prior Publication Data**

US 2010/0193080 A1 Aug. 5, 2010

**Related U.S. Application Data**

(63) Continuation of application No. 11/012,030, filed on Dec. 14, 2004, now Pat. No. 7,717,976.

(51) **Int. Cl.**  
**C21D 7/02** (2006.01)

(52) **U.S. Cl.**  
USPC ..... **148/599**; 148/650; 148/540

(58) **Field of Classification Search** ..... 148/330,  
148/328, 598–603, 540; 420/121, 126–129;  
75/10.15, 10.49, 10.48, 10.46

See application file for complete search history.

(56) **References Cited**

U.S. PATENT DOCUMENTS

3,847,682 A 11/1974 Hook  
3,899,321 A 8/1975 Oliver et al.  
3,928,087 A 12/1975 Hook  
4,168,181 A 9/1979 Perlus et al.  
4,233,065 A 11/1980 Koul  
4,251,268 A 2/1981 Willim

4,339,284 A 7/1982 Hashimoto et al.  
4,375,376 A 3/1983 Rowden et al.  
4,853,032 A 8/1989 Yalamanchili et al.  
5,342,700 A 8/1994 Arnaud et al.  
5,458,699 A 10/1995 Tsukamoto et al.  
5,556,485 A 9/1996 Taylor et al.  
5,595,617 A 1/1997 Tonteling et al.  
5,656,102 A 8/1997 Taylor et al.  
5,656,103 A 8/1997 Roberts

(Continued)

FOREIGN PATENT DOCUMENTS

|    |             |        |
|----|-------------|--------|
| CA | 2293995     | 1/2000 |
| JP | 56-44747    | 4/1981 |
| JP | 2000-144322 | 5/2000 |
| JP | 09287020    | 4/2010 |

OTHER PUBLICATIONS

English abstract of Japanese patent 409078120 to Hisashi Hiraoka et al. Mar. 25, 1997.\*

English abstract of Japanese patent 355125215 to Yasuo Hitomi et al., Sep. 26, 1980.\*

English abstract of Japanese patent 406179054 to Takeshi Sugawara et al., Jun. 28, 1994.\*

(Continued)

*Primary Examiner* — Deborah Yee

(74) *Attorney, Agent, or Firm* — Conley Rose, P.C.; Kristin Jordan Harkins

(57) **ABSTRACT**

A method for making a strain aging resistant steel comprises adding boron to the steel, wherein substantially all of the boron in the steel forms boron nitride. A method for making steel comprises adding a nitride-forming element to the steel to lower the free nitrogen content of the steel to a free nitrogen content specification. A high-carbon steel contains boron nitride, wherein the free nitrogen content of the steel is less than 80 ppm. A strain aging resistant steel wherein the carbon content of the steel is between about 0.54 percent and about 0.75 percent.

**19 Claims, 3 Drawing Sheets**



**U.S. PATENT DOCUMENTS**

|                 |         |                  |
|-----------------|---------|------------------|
| 5,749,981 A     | 5/1998  | Tonteling et al. |
| 5,873,961 A     | 2/1999  | Bhagwat et al.   |
| 6,264,759 B1    | 7/2001  | Bae et al.       |
| 6,322,641 B1    | 11/2001 | Makii et al.     |
| 6,395,107 B1    | 5/2002  | Subramanian      |
| 6,447,622 B1    | 9/2002  | Yamada et al.    |
| 6,537,395 B2    | 3/2003  | Subramanian      |
| 6,596,098 B1    | 7/2003  | Nishida et al.   |
| 6,676,774 B2    | 1/2004  | Matsuoka et al.  |
| 6,692,584 B2    | 2/2004  | Sakata et al.    |
| 6,695,932 B2    | 2/2004  | Kami et al.      |
| 6,702,904 B2    | 3/2004  | Kami et al.      |
| 6,743,306 B2    | 6/2004  | Nakajima et al.  |
| 6,767,417 B2    | 7/2004  | Fujita et al.    |
| 6,800,147 B2    | 10/2004 | Nagao et al.     |
| 6,902,632 B2    | 6/2005  | Kami et al.      |
| 6,949,149 B2    | 9/2005  | Zelin et al.     |
| 2001/0010181 A1 | 8/2001  | Zasowski et al.  |
| 2003/0015263 A1 | 1/2003  | Kami et al.      |
| 2004/0103962 A1 | 6/2004  | Kami et al.      |
| 2004/0105997 A1 | 6/2004  | Kami et al.      |

**OTHER PUBLICATIONS**

English-hand translation of Japanese patent 2000-144322, Sunao Yoshihira et al., May 26, 2000.\*  
English-hand translation of Japanese patent 56-44747, Gennosuke Tenmyo et al., Apr. 24, 1981.\*  
Machine-English translation of Japanese patent 09-287020, Murakami Toshiyuki et al., Nov. 4, 1997.\*  
“Classification of Carbon and Low-Alloy Steels,” Knowledge Article from [www.Key-to-Steel.com](http://www.Key-to-Steel.com), Aug. 16, 2004, <http://key-to-steel.com/ViewArticle.asp?ID=62>, 4 pgs.  
“How Steel is Made,” UK Steel Association, 1999, <http://www.uksteel.org.uk.htm>, 5 pgs.  
“The Metallurgy of Carbon Steel,” Aug. 13, 2004, <http://gowelding.com/met/carbon.htm>, 5 pgs.  
Jones, Jeremy A.T., “Electric Arc Furnace Steelmaking,” American Iron and Steel Institute: Steel Works, Sep. 3, 2004, <http://www.steel.org/learning/howmade/eaft.htm>, 16 pgs.  
Kozak, Bruce, et al., “Continuous Casting of Steel: Basic Principles,” American Iron and Steel Institute: Steel Works, Sep. 20, 2004, <http://www.steel.org/learning/howmade/concast.htm>, 10 pgs.

\* cited by examiner



*Fig. 1*



*Fig. 2*



*Fig. 3*



Fig. 4



Fig. 5

## 1

**METHOD FOR MAKING STRAIN AGING RESISTANT STEEL****CROSS-REFERENCE TO RELATED APPLICATIONS**

This application is a Continuation of and claims benefit under 35 USC §120 to U.S. patent application Ser. No. 11/012,030 entitled "Method for Making Strain Aging Resistant Steel" filed Dec. 14, 2004, now U.S. Pat. No. 7,717,976 which is assigned to the Assignee of the present application and hereby incorporated by reference as if reproduced in its entirety.

**STATEMENT REGARDING FEDERALLY SPONSORED RESEARCH OR DEVELOPMENT**

Not applicable.

**REFERENCE TO A MICROFICHE APPENDIX**

Not applicable.

**BACKGROUND**

The present disclosure relates generally to methods for modifying the chemistry in steel. More specifically, the method relates to forming a strain aging resistant steel by using nitride-forming elements, such as boron, to limit the free nitrogen content in high-carbon steel, or to meet a free nitrogen content specification in either high or low-carbon steel.

Steel is generally classified as either high-carbon steel or low-carbon steel. Generally, low-carbon steel contains less than 0.25 percent carbon, and high-carbon steel contains more than 0.25 percent carbon. Low-carbon steel is tough and ductile and is used for screws, nails, automotive body panels, and similar products that do not have critical strength requirements. Toughness is defined as the capacity of the steel to absorb energy without fracturing. Ductility is defined as the ability of steel to undergo permanent changes in shape without fracturing at room temperature.

High-carbon steel is much harder than low-carbon steel due to the presence of both iron carbide (cementite) and iron that form pearlite in the steel. High-carbon steel is used for manufacturing parts that have critical strength requirements, such as shafts, axles, gears, crankshafts, couplings, forgings, rails, railway wheels, and rail axles. High-carbon steel can be heat-treated to high hardness, but loses its toughness and ductility. Hardness is defined as the degree to which the steel will resist cutting, abrasion, penetration, bending and stretching. High tensile strength typically corresponds with high hardness.

One method for making steel products is by refining iron ore into steel. First, iron ore is mined from the earth and transported to a steel mill. The iron ore is then mixed with limestone and coal and heated in a blast furnace. The blast furnace melts the iron ore and removes most of the impurities from the liquid iron, creating a product called pig iron. The carbon content of the pig iron is too high for most steel products, so the pig iron is either further refined in its liquid form or cast into ingots for later use. In either case, the pig iron must be refined to reduce the carbon content and form usable liquid steel. The liquid steel may then be cast into slabs or billets for later processing into steel products.

A downside to this method for making steel products is the expense associated with mining and refining the iron ore into

## 2

pig iron. One solution is to use direct reduced iron, which is iron ore that has been crushed and refined using large amounts of natural gas. However, the economic attractiveness of direct reduced iron is highly dependent upon the price of natural gas; therefore, direct reduced iron is not always a viable option. Steel mills have found that the use of scrap steel is an attractive alternative to either pig iron or direct reduced iron. The scrap steel is melted into liquid steel using an electric arc furnace or a basic oxygen furnace. The liquid steel can then be cast into slabs or billets. If an electric arc furnace is used, the furnace is charged with the scrap steel, and three graphite electrodes inside the furnace create electric arcs that melt the steel scrap into liquid steel. By contrast, if a basic oxygen furnace is used, the furnace is charged with a mixture of scrap and liquid pig iron, and oxygen is blown into the liquid steel to melt the scrap and purify the steel. The liquid steel is then transferred to a ladle metallurgy furnace (LMF) where the chemistry of the liquid steel is adjusted to meet a steel specification. The liquid steel may then be used to make steel products. The use of scrap steel in an electric arc furnace is typically the most cost-effective method for manufacturing steel products.

A commonly manufactured steel product is steel wire. Steel mills manufacture steel wire by forming a billet, rolling the billet into a steel rod, and then cold drawing the rod to form a wire. Cold drawing is the process of forcing a steel rod through a die to elongate and reduce its diameter. The steel rod is not heated before or as it is being forced through the die, hence the name "cold drawing." When the steel rod exits the die, the rod is called a wire. The cold drawing process may be repeated using increasingly smaller diameter dies to produce a wire of any diameter. The wire may be heat treated after wire drawing for improved mechanical properties. The wire may then be sold as bulk wire or may be formed into wire products, such as lacing wire or springs.

One problem that occurs when wire is cold drawn is strain aging. Strain aging is a condition where the ductility of the steel is reduced such that the steel becomes brittle, and therefore cracks and breaks rather than bends during the subsequent forming process. There are two main types of strain aging: dynamic strain aging and static strain aging. Dynamic strain aging occurs when the rod is cold drawn to form the wire. Static strain aging occurs between the time when the wire is cold drawn and the time when it is formed into a wire product. Strain aging is a significant problem in the steel industry and has been widely discussed in the prior art.

One of the primary causes of both dynamic and static strain aging is the presence of large quantities of "free nitrogen" dissolved within the steel. All of the free nitrogen dissolved within the steel is present as atomic nitrogen. Experiments have shown that when the nitrogen content of steel is greater than about 80 ppm, the steel will exhibit strain aging, and that strain aging is substantially reduced or eliminated when the nitrogen content of steel is below about 65 ppm, about 60 ppm, and preferably about 50 ppm. On an atomic level, strain aging is caused by the relatively small nitrogen atoms impeding the movement of dislocations within the iron atom matrix as the steel passes through the die. It is widely believed that if the movement of free nitrogen within the iron matrix is reduced or "stabilized," then dislocations can move easier within the iron matrix and strain aging will be reduced or eliminated. Therefore, a need exists for a method of making steel in which the free nitrogen in the steel is stabilized, thereby increasing the steel's resistance to strain aging.

Table 1 below outlines the nitrogen content of steel by different processes:

TABLE 1

| Steel Making Process                                | Typical Nitrogen Content |
|-----------------------------------------------------|--------------------------|
| Basic Oxygen Furnace Using Pig Iron and Steel Scrap | 20-40 ppm                |
| Electric Arc Furnace Using Steel Scrap and          | 50-80 ppm                |
| Combinations of Pig Iron and Direct Reduced Iron    |                          |
| Electric Arc Furnace Using Steel Scrap Only         | 50-100 ppm               |

Thus, strain aging is particularly problematic in steel produced using an electric arc furnace because such steel has a higher nitrogen content. This is due, in part, to the use of scrap steel, which has a higher nitrogen content than pig iron or direct reduced iron. As a result, the liquid steel formed from scrap steel has a higher nitrogen content than the liquid steel formed from either pig iron or direct reduced iron. In addition, the electric arc from the electrodes causes molecular nitrogen in the air ( $N_2$ ) to dissociate into atomic nitrogen, which is easily absorbed by the liquid steel. Thus, unless the steel mill implements a nitrogen-reduction process, the nitrogen content of the solidified steel will be even higher than the nitrogen content of the steel scrap used to charge the furnace.

The conventional methods for controlling the nitrogen content of the steel involve the use of additional carbon in the charge, additional oxygen during refining, shielding gases during refining, and/or shrouding equipment during transfer and casting. One of the chemical reactions that occurs in the liquid steel is the interaction of carbon and oxygen, which produces carbon monoxide (CO). Because one of the byproducts of the carbon-oxygen reaction is removal of nitrogen from the liquid steel, the amount of carbon and/or oxygen in the liquid steel can be increased to control the nitrogen content of the steel. The carbon content can be increased by using additional charge carbon, injected carbon, pig iron, or direct reduced iron in the steel. The oxygen content can be increased by adding additional oxygen gas to the liquid steel. In either case, the modified refining process requires more raw materials and/or more expensive raw materials and more processing time than steel production methods in which the nitrogen content is not controlled. An additional method of controlling the nitrogen content of the steel is to use a shielding gas, such as argon, to stir the steel and shield the steel from the nitrogen in the atmosphere. By bubbling the shielding gas through the liquid steel to stir it and covering the surface of the liquid steel with a layer of the shielding gas, the amount of nitrogen the steel absorbs from the atmosphere can be controlled. Moreover, the amount of nitrogen the steel absorbs from the atmosphere can be controlled by using shrouding equipment when transferring the steel between the melting furnace, the LMF, and the caster. Shrouding equipment is also effective at controlling the amount of nitrogen the steel absorbs from the atmosphere when the steel is being cast.

The aforementioned methods for controlling the nitrogen content of the steel are not preferred because they significantly increase the cost of producing the steel and/or substantially reduce the throughput rate of steel production. The use of additional charge and injected carbon and carbon in the form of pig iron and/or direct reduced iron increases the cost of the raw materials. The use of additional oxygen during refining increases the cost of the raw materials and requires additional refining time, thereby decreasing the throughput rate of the steel production. Shielding gases, such as argon, increase the production cost of the steel because the shielding gas is generally not recoverable once used. Finally, the use of

shrouding equipment increases the capital cost of the steel mill, which when amortized over the life of the equipment, increases the production cost of the steel. If a method for reducing the nitrogen content of the steel existed, then the aforementioned methods for controlling the nitrogen content of the steel would be unnecessary. In other words, if a method for reducing the nitrogen in the steel existed, then steel could be produced without regard for its nitrogen content and the nitrogen content of the steel could be reduced using the nitrogen reduction method. Consequently, a need exists for a method of reducing the nitrogen content of steel.

The conventional methods of reducing the nitrogen content of steel are also not preferred due to concerns about the costs and/or lowered productivity associated with these methods.

Another method for limiting the nitrogen content of steel is to refine the steel using a basic oxygen furnace instead of an electric arc furnace. However, basic oxygen furnaces have two disadvantages: they are more expensive to install and operate and they require a charge comprising a mixture of scrap and liquid pig iron. Another method for limiting the nitrogen content in steel is to use a vacuum degasser on the LMF. A vacuum degasser operates under the principle that the nitrogen in the steel is in equilibrium with the nitrogen in the air above the liquid steel. The vacuum degasser lowers the pressure of the air (i.e. creates a vacuum) above the liquid metal, thereby lowering the partial pressure of the nitrogen in the air and causing the nitrogen in the steel to transfer from the liquid phase to the gaseous phase. However, vacuum-degassing equipment is expensive to purchase, install, and operate. The vacuum degassing process is also relatively time consuming because of the slowness in removing nitrogen from liquid steel under vacuum, which lowers the throughput rate of the steel mill. Consequently, a need exists for a simple, quick, and relatively inexpensive method to reduce the free nitrogen content in steel, thereby creating a strain aging resistant steel.

#### SUMMARY OF THE INVENTION

The present invention is directed to a method for making a strain aging resistant steel comprising adding boron to the steel wherein substantially all of the boron in the steel forms boron nitride, stabilizing the free nitrogen in the steel. In an embodiment, the method further comprises analyzing the chemistry of the steel, deoxidizing the steel, adding boron to the steel after the steel has been deoxidized, casting the steel into a billet, rolling the billet into a rod, and cold drawing the rod into a wire. In an embodiment, the pre-processed steel has a nitrogen content of at least about 50 ppm prior to adding the boron to the steel. In various embodiments, the resultant steel contains at least about 0.25 percent carbon, less than about 30 ppm oxygen, and less than about 80 ppm free nitrogen. The boron may be added to the steel in a stoichiometric amount to stabilize the free nitrogen in the steel such that the steel meets a free nitrogen content specification of less than about 80 ppm. The boron may be added to the steel in the form of a bulk boron alloy, a wire with a steel sheath and a boron core, or a boron powder.

In another aspect, the present invention is directed to a method for making steel comprising adding a nitride-forming element to the steel to lower the free nitrogen content of the steel to a free nitrogen content specification to make the steel strain aging resistant. In an embodiment, the nitride-forming element is boron and the nitride compound is boron nitride. Alternatively, the nitride-forming element may be selected from the group consisting of aluminum, vanadium, niobium, and titanium; and the nitride compound may be selected from

the group consisting of aluminum nitride, vanadium nitride, niobium nitride, and titanium nitride. The free nitrogen content specification may be less than about 80 ppm. In an embodiment, the method further comprises casting the steel into a billet, rolling the billet into a rod, and cold drawing the rod into a wire. In various embodiments, the steel has a free nitrogen content of at least about 50 ppm prior to adding the boron to the steel, contains at least about 0.25 percent carbon, and contains less than about 30 ppm oxygen. In an embodiment, substantially all of the boron in the steel exists as boron nitride. The boron may be added to the steel in the form of a bulk boron alloy or a wire with a steel sheath and a boron core.

In yet another aspect, the present invention comprises a high-carbon, strain aging resistant steel containing boron nitride; wherein the free nitrogen content of the steel is less than about 80 ppm. In an embodiment, substantially all of the boron in the steel exists as boron nitride. In various embodiments, the steel has a free nitrogen content of at least about 50 ppm prior to adding the boron to the steel, contains at least about 0.25 percent carbon, and contains less than about 30 ppm oxygen. The final steel may contain less than about 65 ppm free nitrogen.

In still another aspect, the present invention comprises a strain aging resistant steel wherein the carbon content of the steel is between about 0.54 percent and about 0.75 percent. In an embodiment, substantially all of the boron in the steel exists as boron nitride. In various embodiments, the steel contains less than about 30 ppm oxygen and less than about 80 ppm free nitrogen.

#### BRIEF DESCRIPTION OF THE DRAWINGS

For a more complete understanding of the present invention, and for further details and advantages thereof, reference is now made to the accompanying drawings, in which:

FIG. 1 is a block diagram of one embodiment of a method for making strain aging resistant steel;

FIG. 2 is a side view of one embodiment of an electric arc furnace used to implement the method of FIG. 1 making strain aging resistant steel;

FIG. 3 is a side view of one embodiment of a ladle metallurgy furnace (LMF) used to implement the method of FIG. 1 for making strain aging resistant steel;

FIG. 4 is a side view of one embodiment of a continuous caster used to implement the method of FIG. 1 for making strain aging resistant steel; and

FIG. 5 is a cross-sectional view of one embodiment of a die used to implement the method of FIG. 1 for making strain aging resistant steel.

#### DETAILED DESCRIPTION OF THE INVENTION

FIG. 1 depicts a block diagram of the major steps comprising one embodiment of a method 10 for making strain aging resistant steel. The method 10 comprises charging an electric arc furnace with scrap steel 15, melting the scrap steel 20, transferring the liquid steel to a ladle metallurgy furnace (LMF) 22, analyzing the chemistry of the steel 25, modifying the chemistry of the steel 30, deoxidizing the steel 35, and adding boron to the steel 40. The method 10 further comprises transferring the liquid steel to a continuous caster 42, casting it into billets 45, rolling the billets into rods 50, cold drawing the rods into wire 55, and optionally heat treating the wire 60. Each of these steps is described in greater detail below.

FIG. 2 is an illustration of one embodiment of an electric arc furnace 100 used to melt the scrap steel into liquid steel per step 20 of FIG. 1. Although the specific design varies from

one steel mill to another, the electric arc furnace 100 generally comprises a shell 118 and a roof 116. Both the shell 118 and the roof 116 may be manufactured of steel plate, the interior of which is lined with refractory 119 and/or water cooled panels (not shown). The roof 116 contains three graphite electrodes 102, each of which are connected to an electrical power source (not shown). The electrodes 102 generate electric arcs 104 between each other. A plurality of supports 112 allow the roof 116 to be retracted with respect to the shell 118. The shell 118 contains a tap 114 that may be opened to drain the liquid steel out of the electric arc furnace 100.

The electric arc furnace 100 operates to produce batches of liquid steel. The process usually begins with the retraction of the roof 116 away from the shell 118. If necessary, the interior of the electric arc furnace 100 is inspected and repaired during this time. The electric arc furnace 100 is then charged with scrap steel per step 15 of FIG. 1. If desired, fluxes, charge carbon, and alloying metals (not shown), such as molybdenum, manganese, and chromium, are added to the scrap steel to make the composition of the liquid steel closer to the final steel specification. When the electric arc furnace is sufficiently charged with scrap steel, the roof 116 is lowered to be positioned on top of the shell 118 and electric power is supplied to the electrodes 102. The arcs 104 melt the scrap steel into liquid steel 106 per step 20 of FIG. 1. As the scrap steel melts into liquid steel 106, a layer of slag 110 forms between the liquid steel 106 and the gases 108 in the electric arc furnace 100. If the scrap steel charge contains alloying metals, the alloying metals melt with the scrap steel. Optionally, additional charges of scrap steel may be added to the electric arc furnace 100. When the scrap steel, additional charges, and/or alloying metals are completely melted and refined into liquid steel 106, the electric arc furnace 100 is tapped by draining the liquid steel out of the tap 114. Additives including fluxes, carbon, and alloys may be added during the tapping step. The semi finished liquid steel 106 is then transferred per step 22 of FIG. 1 to the LMF 120 shown in FIG. 3, where the liquid steel is further refined to the final specification.

It should be understood that the method for making strain aging resistant steel is not to be limited to the use of scrap steel melted in an electric arc furnace 100. Instead, the method may also include the use of steel scrap, pig iron, direct reduced iron, and combinations thereof in an electric arc furnace, a basic oxygen furnace, or other types of furnaces.

FIG. 3 is an illustration of a LMF 120 used to modify the chemistry of the steel, analyze the chemistry of the steel, deoxidize the steel, and add boron to the steel according to steps 25, 30, 35, and 40 of FIG. 1. Much like the electric arc furnace 100, the LMF 120 generally comprises a ladle shell 126 and a roof 128. The LMF 120 also comprises an alloy addition system, a gaseous or electromagnetic stirring system, and a wire injection system. Samples for chemical analysis are taken with disposable probes that are inserted into the liquid steel 106. The LMF 120 is also equipped with graphite electrodes 102 for the purpose of heating the liquid steel 106, and a porous plug arrangement (not shown) for bubbling gas through the liquid steel 106 to stir and mix it. The LMF 120 may also comprise additional apparatuses other than those described herein.

After the liquid steel 106 is transferred from the electric arc furnace 100 into the LMF 120 per step 22 of FIG. 1, the chemical composition of the liquid steel 106 is analyzed in accordance with step 25 of FIG. 1. The chemical composition identifies the content of several important elements in the steel, including: carbon, manganese, phosphorous, sulfur, silicon, copper, nickel, chromium, molybdenum, aluminum,

nitrogen, boron, vanadium, and niobium. Oxygen is measured with immersion probes. The LMF operator uses the chemical composition of the liquid steel 106 to determine which refining processes to implement on the liquid steel 106 to meet a steel specification. While there are several steel specifications, the most widely recognized specifications are those provided by the American Society for Testing and Materials (ASTM) and the American Iron and Steel Institute (AISI). Customer specifications are also frequently used. The method for making strain aging resistant steel includes steel specifications other than the steel specifications described herein and the method is not limited to any of the aforementioned steel specifications.

After the chemical composition of the steel has been analyzed, the chemical composition of the liquid steel 106 may be modified by adding alloys in bulk or as wire, carbon, and fluxes, to the liquid steel or implementing various processes on the steel in accordance with step 30 of FIG. 1. For example, if the manganese content of the steel is too low for the steel specification, manganese may be added to the liquid steel 106 as a ferro alloy or as a pure metal. As another example, if the carbon content of the steel is too low, carbon can be added as a cored wire or in bulk form. As the chemistry of the liquid steel 106 is being modified, the steel mill may periodically re-analyze and monitor the chemical composition of the steel. The method for making strain aging resistant steel also includes chemical content additions and processes other than those described herein, and the method for is not limited to any of the aforementioned additions and processes.

After the chemical composition of the steel has been modified, the steel mill deoxidizes the steel in accordance with step 35 of FIG. 1. Deoxidizers such as silicon or manganese reduce the oxygen content to a level where no reaction occurs between carbon and oxygen during solidification. In the preferred deoxidation process, silicon, calcium, or a combination is added to the steel until the oxygen content of the steel is reduced to a specification level, such as less than about 100 parts per million (ppm). In an embodiment, the oxygen content is reduced to less than about 30 ppm. In another embodiment, the oxygen content is reduced to less than about 20 ppm so that when a nitride-forming element is added to the steel, the nitride-forming element reacts with the free nitrogen to form nitrides instead of reacting with the oxygen to form oxides. The method for making strain aging resistant steel also includes steel deoxidation methods other than those described herein, and the method is not limited to the aforementioned steel deoxidation methods.

After the steel has been deoxidized, the steel mill adds a nitride-forming element to stabilize the free nitrogen in the steel in accordance with step 40 of FIG. 1. Several nitride-forming elements are suitable for making strain aging resistant steel, including: boron, aluminum, titanium, vanadium, and niobium (also called columbium). Generally, the nitride-forming element reacts with free nitrogen to form a binary molecule (i.e.  $B+N \rightarrow BN$ ). However, some nitride-forming elements, such as vanadium, also form more complex molecules (i.e.  $4V+N \rightarrow V_4N$ ). Selection of a specific nitride-forming element varies from application to application depending upon the end-use for the steel, and upon the carbon, nitrogen, and oxygen content in the steel, which is important because some nitride-forming elements prefer to form carbides and oxides instead of nitrides. The formation of carbides and oxides does not necessarily have an adverse affect on the steel, but a greater amount of nitride-forming element is required to reduce the free nitrogen content to a specified level when the nitride-forming element also forms carbides and oxides. The method for making strain aging

resistant steel also includes nitride-forming elements other than those described herein, and the method is not limited to the aforementioned nitride-forming elements.

In another embodiment, boron is the selected nitride-forming element because boron prefers to form nitrides over oxides and carbides, and the boron nitride is not harmful to the finished wire. In more detail, many nitride-forming elements, such as aluminum, prefer to form oxides instead of nitrides. Because most steel specifications do not have a lower limit for oxygen content, the oxide formation can be controlled by reducing or eliminating the oxygen content in the steel during the deoxidation process. However, nitride-forming elements with a high oxygen affinity, such as aluminum, will seek to bond with oxygen and further deoxidize the steel rather than bond with nitrogen and stabilize the free nitrogen in the steel.

Likewise, some nitride-forming elements, such as titanium, prefer to form carbides over nitrides. Because steel specifications set upper and lower limits for carbon content, the formation of carbides cannot be controlled by simply limiting the carbon content in the steel. Thus, in high-carbon steels, nitride-forming elements with an affinity for carbides are not preferred because such elements will bond with carbon to form carbides instead of bonding with free nitrogen to form nitrides.

Accordingly, nitride-forming elements, such as boron, having a strong affinity for forming nitrides over oxides or carbides are preferred in high-carbon steels, and are also suitable for steel with any carbon content. For example, even in high-carbon steel, substantially all of the boron will form boron nitride with minimal boron carbide formation. Similarly, in higher oxygen steel, most of the boron will form boron nitride with minimal boron oxide formation. Consequently, boron is an excellent nitride-forming element because boron has a strong preference for forming nitrides over oxides or carbides.

Boron is also an advantageous nitride-forming element because of its cost and the stoichiometric efficiency with which boron forms nitrides. The amount of nitride-forming element required to bond with a specified amount of free nitrogen is dependent upon the atomic weight of nitrogen, the atomic weight of the nitride-forming element, and the coefficients of the balanced chemical reaction. The content of the nitride-forming element can be calculated using the following equation:

$$\text{Content}_{NFE} = \frac{[(\text{Content}_N) \times (\text{MW}_{NFE})] \times (\text{Coefficient}_{NFE})}{[(\text{MW}_N) \times (\text{Coefficient}_N)]} \quad (1)$$

Where:

“Content<sub>NFE</sub>” is the amount of nitride-forming element required to stabilize the nitrogen in the steel (in ppm);

“MW<sub>NFE</sub>” is the molecular weight of the nitride-forming element (in grams per mole);

“Coefficient<sub>NFE</sub>” is the coefficient of the nitride-forming element reactant in the stoichiometrically balanced reaction equation;

“Content<sub>N</sub>” is the amount of free nitrogen to be removed from the steel (in ppm);

“MW<sub>N</sub>” is the molecular weight of nitrogen (in grams per mole); and

“Coefficient<sub>N</sub>” is the coefficient of the nitrogen reactant in the balanced reaction equation. Applying the above equation to the boron nitride reaction ( $B+N \rightarrow BN$ ), in which the boron and nitrogen coefficients are both 1, it is evident that only 0.77 ppm of boron is required to react with 1 ppm of free nitrogen. By contrast, 3.42 ppm of titanium and 6.64 ppm of niobium, respectively, would be required to react with the same 1 ppm

of free nitrogen. Because boron has the lowest molecular weight, less boron is required as compared to other nitride-forming elements. Boron is also less expensive than other nitride-forming elements, such as titanium and niobium. Consequently, the stoichiometric efficiency with which boron forms nitrides, coupled with the cost of boron, makes boron an excellent nitride-forming element for the method of making strain aging resistant steel.

The decision regarding whether to add a nitride-forming element, such as boron, to the liquid steel is based upon the nitrogen content of the steel. The amount of nitrogen allowed in the steel varies from specification to specification and is commonly based upon the desired physical properties of the resultant steel. In some types of steel, the steel specification limits the nitrogen content to less than about 80 ppm nitrogen. Thus, if the steel has a nitrogen content of less than about 80 ppm, then there is no need to add a nitride-forming element to the steel. Further, many steel specifications limit the nitrogen content to a maximum of about 65 ppm, while others limit the nitrogen content to a maximum of about 60 ppm or a maximum of about 50 ppm. Thus, it may be necessary to limit the nitrogen content of the steel to about 80 ppm, about 65 ppm, about 60 ppm, or about 50 ppm. Alternatively, the steel mill can limit the nitrogen content to any other amount as described in a specification and/or customer requirement. The liquid steel will absorb an incidental amount of nitrogen, usually between about 5 ppm and about 15 ppm, between the time the chemical composition is analyzed and the time the liquid steel solidifies. This nitrogen absorption is taken into account when deciding whether or not to add the nitride-forming element to the liquid steel. Because the liquid steel acquires the majority of its nitrogen from either the steel charge or the dissociation of molecular nitrogen by the electricity, if the nitrogen content of the steel does not exceed the nitrogen content in the specification minus the expected nitrogen absorption, then there is generally no need to add a nitride-forming element to the steel. Instead, the steel is sent directly to the caster.

In a majority of cases, particularly when an electric arc furnace is used to melt scrap steel, the nitrogen content of the steel exceeds about 80 ppm, so there is a need to stabilize the free nitrogen in the steel by adding a nitride-forming element, such as boron, to the steel. The amount of nitride-forming element to add to the steel is based upon the amount of nitrogen to be stabilized, which may be calculated using the following equation:

$$\text{Content}_N \text{ to be Stabilized} = (\text{Content}_N \text{ of the Steel} - \text{Content}_N \text{ in the Specification}) \quad (2)$$

Where:

“Content<sub>N</sub> to be Stabilized” is the amount of free nitrogen in the steel that needs to be stabilized to bring the steel into conformance with the specification;

“Content<sub>N</sub> of the Steel” is the amount of free nitrogen in the steel before adding any nitride-forming elements; and

“Content<sub>N</sub> in the Specification” is the maximum free nitrogen content of the specification. By using the “Content<sub>N</sub> to be Stabilized” in equation 2 as the “Content<sub>N</sub>” in equation 1, the amount of nitride-forming element required to bring the steel into conformance with the specification can be determined. For example, if the nitrogen content of the steel is 100 ppm, the nitrogen specification is 60 ppm maximum, and boron is the nitride-forming element, then 30.9 ppm of boron (30.9 milligrams of boron per kilogram of steel) should be added to the steel. Because the liquid steel tends to absorb some free nitrogen (typically 5-15 ppm) between the chemical composition analysis in the LMF and solidification of the steel, an

additional 5-15 ppm of free nitrogen in the steel should be stabilized to ensure compliance with the steel specification. For example, if the nitrogen content of the steel is 100 ppm, the nitrogen specification is 60 ppm maximum, an additional 10 ppm of nitrogen is to be stabilized, and boron is the nitride-forming element, then 38.6 ppm of boron (38.6 milligrams of boron per kilogram of steel) should be added to the steel. Thus, equation 1 and equation 2 may be used to calculate the amount of nitride-forming element to add to the steel 10 regardless of the nitride-forming element selected, the nitrogen content of the steel prior to adding the nitride-forming element, or the nitrogen content of the steel specification.

The nitride-forming element is added to the liquid steel in a variety of forms. For example, using boron as the nitride-forming element, the boron may be added as a bulk ferro-boron alloy, or injected into the liquid steel as a boron powder or as a steel sheathed wire with a ferro-boron powder core. The wire injection method is advantageous because the wire may be injected directly into the liquid steel using a wire feeder (not shown), which leads to better mixing of the boron with the steel, and thus a more complete reaction between the boron and the free nitrogen. The method for making strain aging resistant steel also includes methods for adding nitride-forming elements to liquid steel by processes other than those described herein, and the method is not limited to the aforementioned processes for adding nitride-forming elements to liquid steel.

After the nitride-forming element has been added to the liquid steel and the free nitrogen stabilized, the liquid steel is transferred to a caster for casting in accordance with steps 42 and 45 of FIG. 1. FIG. 4 is an illustration of one embodiment of a continuous caster 130 suitable for implementing the method for making strain aging resistant steel. Although the method for making strain aging resistant steel may utilize a batch casting process in which the liquid steel is poured into stationary molds to form ingots, continuous casting is more efficient. As depicted in FIG. 4, the liquid steel 106 is poured from the LMF (not shown) into a tundish 132. The tundish 132 is essentially an open-topped tank that feeds the liquid steel 106 into one or more mold(s) 134 at a regulated rate. The tundish 132 is designed to continuously supply liquid steel 106 to the mold(s) 134 at a specific flow rate through nozzles in the bottom of the tundish 132. Cooling water (not shown) flows through the mold(s) 134 and cools the exterior of the mold(s) 134 to a temperature below the solidification temperature of the steel. The mold(s) 134 is constructed of a heat conductive material, preferably copper, and consequently the interior of the mold(s) 134 cools the exterior of the liquid steel 106, thereby transforming it into a steel shell with a liquid steel core. As the steel continues to move down through the caster 130, spray water directly on the outer shell continues to cool the steel until the liquid core solidifies into solid steel 136. The solid steel 136 then passes through a straightener 135 that straightens out the arc shape that the solid steel 136 acquired during casting. The straightened steel 136 is cut by a torch 137, thereby forming a plurality of billets 138. Alternatively, the casting process can produce shapes other than billets, such as blooms, rounds, beam blanks, conventional slabs, or thin slabs. The method for making strain aging resistant steel also includes casting processes other than those described herein, and the method is not limited to the aforementioned casting processes.

After the billets 138 are formed, the billets 138 are rolled into rods at a rolling mill in accordance with step 50 of FIG. 1. The billets 138 produced by the caster 130 are square, rectangular, or round in cross-section, and are large in comparison to wire diameters. However, the dies used to draw the

## 11

wire are small round-shaped and wear prematurely unless round-shaped rods are inserted into the dies. Therefore, the square or rectangular billets 138 must be reshaped into rods with a much smaller circular cross-section. A rolling mill is a machine or group of machines that works the rectangular billets 138 into round bars by rolling the billets 138 under pressure until the billets 138 are much reduced in size and become round. The rolling process is done hot wherein the temperature exceeds the recrystallization temperature of the steel. Hot rolled rods are beneficial because the steel does not strain harden during the rolling process. The method for making strain aging resistant steel also includes rolling processes other than those described herein, and the method is not limited to the aforementioned rolling processes.

After the billets 138 are rolled into rods, the rods are cold drawn through a series of dies to produce drawn wire in accordance with step 55 of FIG. 1. FIG. 5 is an illustration of a die 140, comprising an inlet 142, a throat 144, and an outlet 146. As depicted in FIG. 5, the inlet 142 is sized to accept rods 139 of various diameters,  $d_1$ . The inlet 142 partially constricts larger diameter rods 139; however, the majority of the constricting work is performed by throat 144. The throat 144 constricts the rod 139 down to a wire 148 with a diameter  $d_2$ . As the rod 139 is constricted, the iron atoms in the steel move along slip planes by dislocation movement and reorganize themselves into the smaller diameter wire 148. The constricting process also causes elongation of the steel such that the wire 148 exiting the die 140 is substantially longer than the rod 139 fed into the die 140. The outlet 146 of the die 140 includes a constant diameter section 147 and an expanding diameter section 149 which allows the steel to stabilize before exiting the die 140. If desired, a plurality of dies 140 may be implemented such that the process of drawing the rod 139 into the wire 148 occurs in a plurality of incremental steps. The wire 148 may then be spooled for sale or further processing. The method for making strain aging resistant steel also includes cold working and drawing processes other than those described herein, and the method is not limited to the aforementioned drawing processes.

After the wire 148 has been drawn, the wire 148 may optionally be heat treated in accordance with step 60 of FIG. 1. The process gives the wire 148 greater yield strength, but also makes the wire 148 more brittle and susceptible to break-

## 12

ing. The steel wire 148 containing the nitride-forming element is resistant to strain aging regardless of whether the wire 148 is heat treated or not. Thus, the decision regarding whether to heat treat the wire 148 depends upon the individual application for the wire 148. If the wire 148 is to be heat treated, one heat treating process comprises holding the wire at a temperature between about 450° F. and about 650° F. for about 10 to 20 minutes. The method for making strain aging resistant steel also includes heat-treating processes other than those described herein, and the method is not limited to the aforementioned heat treating processes.

After the wire 148 has been drawn and optionally heat treated, the wire 148 may be used for a variety of purposes. Generally, the diameter of the wire 148 governs its application. For example, wire that is about 0.050 inches in diameter is suitable for use as lacing wire for mattresses, and wire between about 0.007 inches and 0.014 inches in diameter is suitable for use as tire cords in pneumatic tires for vehicles. The wire 148 can also be formed into different shapes, such as helical shapes or springs. The method for making strain aging resistant steel also includes wire uses other than those described herein, and the method is not limited to the aforementioned wire uses.

## EXAMPLE

The method for making strain aging resistant steel was implemented in a steel mill that produced wire according to the process of FIG. 1, including the heat treating step 60. The wire previously produced by the steel mill was 0.050 inch diameter lacing wire that exhibited strain aging. The lacing wire would frequently break when used to assemble mattress components. Twenty-six heats (individual batches of refined steel from a furnace) were made using the method of FIG. 1 making strain aging resistant steel. Boron was added to bring the steel into conformance with a specified free nitrogen content of 80 ppm maximum in the finished steel wire. Previous experiments had shown that the steel absorbed less than 20 ppm of free nitrogen between the LMF and the finished product. Therefore, in cases where the LMF nitrogen content was less than about 60 ppm, little or no boron was added to the LMF to stabilize the free nitrogen. Table 2 below shows the results of the experiment:

TABLE 2

| Heat # | Carbon Content (%) | LMF Nitrogen Content (ppm) | Boron Added to LMF (ppm) | Final Nitrogen Content (ppm) | Stabilized Nitrogen in the form of BN (ppm) | Free Nitrogen (ppm) |
|--------|--------------------|----------------------------|--------------------------|------------------------------|---------------------------------------------|---------------------|
| 1      | 0.66               | 51                         | 0                        | 69                           | 0                                           | 69                  |
| 2      | 0.69               | 61                         | 6                        | 63                           | 8                                           | 55                  |
| 3      | 0.67               | 59                         | 0                        | 69                           | 0                                           | 69                  |
| 4      | 0.68               | 59                         | 0                        | 72                           | 0                                           | 72                  |
| 5      | 0.70               | 68                         | 9                        | 76                           | 11                                          | 65                  |
| 6      | 0.71               | 75                         | 13                       | 86                           | 17                                          | 69                  |
| 7      | 0.72               | 65                         | 16                       | 71                           | 20                                          | 51                  |
| 8      | 0.75               | 66                         | 6                        | 68                           | 8                                           | 60                  |
| 9      | 0.73               | 56                         | 0                        | 77                           | 0                                           | 77                  |
| 10     | 0.77               | 61                         | 0                        | 64                           | 0                                           | 64                  |
| 11     | 0.59               | 76                         | 20                       | 78                           | 25                                          | 53                  |
| 12     | 0.58               | 59                         | 0                        | 61                           | 0                                           | 61                  |
| 13     | 0.59               | 68                         | 15                       | 78                           | 19                                          | 59                  |
| 14     | 0.57               | 52                         | 0                        | 71                           | 0                                           | 71                  |
| 15     | 0.57               | 53                         | 0                        | 71                           | 0                                           | 71                  |
| 16     | 0.57               | 57                         | 1                        | 58                           | 1                                           | 57                  |
| 17     | 0.56               | 50                         | 0                        | 68                           | 0                                           | 68                  |
| 18     | 0.61               | 68                         | 11                       | 69                           | 14                                          | 55                  |
| 19     | 0.60               | 76                         | 4                        | 74                           | 5                                           | 69                  |
| 20     | 0.63               | 58                         | 1                        | 75                           | 1                                           | 74                  |

TABLE 2-continued

| Heat # | Carbon Content (%) | LMF Nitrogen Content (ppm) | Boron Added to LMF (ppm) | Final Nitrogen Content (ppm) | Stabilized Nitrogen in the form of BN (ppm) | Free Nitrogen (ppm) |
|--------|--------------------|----------------------------|--------------------------|------------------------------|---------------------------------------------|---------------------|
| 21     | 0.57               | 67                         | 11                       | 72                           | 14                                          | 58                  |
| 22     | 0.58               | 61                         | 1                        | 63                           | 1                                           | 62                  |
| 23     | 0.56               | 56                         | 0                        | 61                           | 0                                           | 61                  |
| 24     | 0.55               | 64                         | 1                        | 63                           | 1                                           | 62                  |
| 25     | 0.56               | 55                         | 0                        | 71                           | 0                                           | 71                  |
| 26     | 0.54               | 52                         | 0                        | 65                           | 0                                           | 65                  |

The steel wire produced in all twenty-six heats did not exhibit strain aging, thereby supporting the conclusion that the addition of a nitride-forming element, such as boron, stabilizes the free nitrogen to substantially reduce or eliminate the effects of strain aging. In addition, the experiment shows that the method of making strain aging resistant steel is effective to produce steel conforming to a free nitrogen specification of 15 65 ppm, 60 ppm, and/or 50 ppm.

The method for making strain aging resistant steel may be applied to steel containing any level of carbon, but high-carbon steel, that is, steel containing at least about 0.25 percent carbon, is more susceptible to strain aging. Steel with a carbon content below 0.25 percent tends to be soft and ductile and generally does not exhibit harmful strain aging. If steel containing less than about 0.25 percent carbon exhibits strain aging, the method for making strain aging resistant steel may be utilized on the steel. However, the advantageous effects of the method for making strain aging resistant steel will generally be most appreciated in steel containing more than about 0.25 percent carbon. Most preferably, the method for making strain aging resistant steel is used on steel with a carbon content between about 0.54 percent and 0.77 percent, as illustrated in Table 2. Steel with a carbon content between about 0.54 percent and 0.77 percent is useful for making 20 0.050-inch lacing wire for mattresses. The method for making strain aging resistant steel may also be used on steel containing more than 0.77 percent carbon, if desired.

While several embodiments of the invention have been shown and described herein, modifications thereof may be made by one skilled in the art without departing from the spirit and the teachings of the invention. The embodiments described herein are provided for purposes of example only and are not intended to be limiting. Many variations, combinations, and modifications of the invention disclosed herein are possible and are within the scope of the invention. Accordingly, the scope of protection is not limited by the description set out above but is defined by the claims which follow, that scope including all equivalents of the subject matter of the claims.

What is claimed is:

1. A method for making a strain aging resistant high carbon spring steel with carbon content between 0.54 and 0.77% for wire drawing comprising:  
setting a free nitrogen content specification, wherein the free nitrogen content specification requires a free nitrogen content that is no more than a set ppm number but no less than 20 ppm below the set ppm number, and the set ppm number is between about 50 ppm and about 80 ppm;  
adding nitride-forming element to a pre-processed steel to form a resultant steel with a free nitrogen content in 55 60 65 conformance with the free nitrogen content specification;

15 forming the resultant steel into a billet, rolling the billet into a rod, and cold drawing the rod into wire;  
wherein:

substantially all of the nitride-forming element in the resultant steel exists as a nitride compound;  
the rod is cold drawn into wire without heat treatment; and the resultant high carbon spring steel is strain aging resistant.

2. The method of claim 1 wherein the nitride-forming element is selected from the group consisting of aluminum, vanadium, niobium, titanium, and boron.

3. The method of claim 1 therein only a single nitride-forming element is added to the pre-processed steel, and the nitride-forming element is boron.

4. The method of claim 3 wherein boron is added in an amount less than about 20 ppm.

5. The method of claim 2 further comprising: analyzing the chemistry of the pre-processed steel; deoxidizing the pre-processed steel; and adding nitride-forming element to the pre-processed steel after the pre-processed steel has been deoxidized; wherein the pre-processed steel contains less than about 30 ppm oxygen after the pre-processed steel has been deoxidized.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505

**15**

steel into wire, wherein the resultant steel is drawn into wire without heat treatment.

9. The method of claim 8 wherein the resultant steel contains between about 0.54 and 0.77 percent carbon.

10. The method of claim 8 wherein the set ppm number is about 80, and the free nitrogen content of the resultant steel is between about 50 and about 80.

11. The method of claim 8 wherein the set ppm number is about 65, and the free nitrogen content of the resultant steel is between about 50 and about 65.

12. The method of claim 8 wherein the set ppm number is about 50, and the free nitrogen content of the resultant steel is between about 30 and about 50.

13. The method of claim 8 further comprising determining an amount of nitride-forming element to add to the pre-processed steel based on the nitrogen content of the pre-processed steel and the expected free nitrogen absorption prior to solidification of the resultant steel.

14. The method of claim 13 wherein the expected free nitrogen absorption is between about 5 ppm and about 20 ppm.

15. A method for making a strain aging resistant steel for wire drawing having carbon content between about 0.54 and 0.77 percent comprising:

setting a free nitrogen content specification, wherein the free nitrogen content specification requires a free nitrogen content no more than a set ppm number, and the set ppm number is between about 50 ppm and about 80 ppm;

5

10

15

20

25

**16**

adding nitride-forming element to a pre-processed steel to form a resultant steel with a free nitrogen content in conformance with the free nitrogen content specification;

wherein:

nitride-forming element is only added in an amount sufficient to form resultant steel having a free nitrogen content no more than 20 ppm below the set ppm number, taking into account the nitrogen content of the pre-processed steel and the expected free nitrogen absorption prior to solidification of the resultant steel; substantially all of the nitride-forming element in the resultant steel exists as a nitride compound; and the resultant steel is strain aging resistant; and further comprising forming the resultant steel into a billet, rolling the billet into a rod, and cold drawing the rod into wire, wherein the wire has a diameter of about 0.05 inch, and the rod is cold drawn into wire without heat treatment.

16. The method of claim 15 wherein nitride-forming element comprises boron.

17. The method of claim 16 wherein the pre-processed steel is derived from an electric arc furnace.

18. The method of claim 17 wherein the pre-processed steel contains less than about 30 ppm oxygen.

19. The method of claim 17 wherein the pre-processed steel has a free nitrogen content above the set ppm number of the free nitrogen content specification.

\* \* \* \* \*

UNITED STATES PATENT AND TRADEMARK OFFICE  
**CERTIFICATE OF CORRECTION**

PATENT NO. : 8,419,870 B2  
APPLICATION NO. : 12/761255  
DATED : April 16, 2013  
INVENTOR(S) : C. Larry Coe and Alan T. Gorton

Page 1 of 1

It is certified that error appears in the above-identified patent and that said Letters Patent is hereby corrected as shown below:

In the Claims

Column 14, Line 65, after "resultant" insert --steel--.

Signed and Sealed this  
Twenty-fifth Day of June, 2013



Teresa Stanek Rea  
*Acting Director of the United States Patent and Trademark Office*